

## 1

2,701,213

## PROCESS FOR RECLAIMING ASPHALTIC PAVEMENT AND A COMPOSITION SO FORMED

Charle A. Neville, Sacramento, Calif., assignor to Reclaimix, Inc., San Jose, Calif., a corporation of California

No Drawing. Application December 16, 1950,  
Serial No. 201,227

5 Claims. (Cl. 106—278)

This invention relates to asphaltic compositions and has particular reference to bituminous or asphaltic compositions for use in road building or the like, and to processes for making such compositions.

One of the principal objects of my invention is to provide a novel process for salvaging or reclaiming the dry and brittle asphaltic surface material of roads, landing field runways and the like and restoring the material to its original condition.

Another important object of my invention is to provide a novel process for reclaiming asphaltic material with which process roads and the like may be rebuilt and restored to a condition equal to that of a new surface, but at a cost considerably less than the cost of building a new surface.

Another object of my invention is to provide a novel process for reclaiming asphaltic surface material which includes the steps of removing the old surface, reducing the particles to size, mixing with the recovered material a quantity of a softener or conditioner to a consistency equal to that of a new asphaltic surface.

Another object of my invention is to provide novel compositions of matter having an asphalt binder and adapted for use in road surfacing and the like.

Another object of my invention is to provide novel asphaltic compositions for use in road building and the like, which compositions may be applied at ordinary temperatures without the use of the heat which is conventionally required in order to render the asphalt workable.

Other objects and advantages of my invention it is believed will be readily apparent from the following detailed description of preferred embodiments thereof.

In the past, attempts have been made to reclaim old and worn asphalt or bituminous pavements. One method has been to rip up the old surface and reduce the material in size by means of various mechanical crushers or grinders and to blend with this material an added quantity of asphalt cutback. This mixture was then relaid as

A class of softeners or conditioners for asphalt has been discovered which act as such without stripping the asphalt from the aggregate, and in addition they leave a desirable residue of nonasphaltic flux oils in the surface.

5 These flux oils blend with the oxidized residual asphalt in the surface material to be treated and revitalize the asphalt, restoring its original quality of resiliency and flexibility.

These conditioners, which may be employed in the process described hereinafter, are of several important classifications, dependent upon their sources. The essential criterion upon which the broad classification is based is that the conditioner must contain a minimum of 40% aromatics. Preferably the conditioner has a boiling range of from 400 to 750° F., since such materials not only provide optimum softening for asphalt surfaces but also restore thereto the flux oil fractions which have disappeared for one reason or another from the asphalt during its aging or weathering.

Conditioners within this boiling range and having more than about 40% aromatics include especially catalytically cracked gas oil, coal tar extracts, highly thermally cracked oils and extracts of the Edeleanu type. The latter type of extracts includes those prepared by the extraction of petroleum fractions with solvents such as liquid sulfur dioxide, furfural, phenol, aniline and similar well-known solvents which have a preferential solubility of aromatic constituents.

Catalytically cracked gas oil is a preferred type of conditioner since it contains not only a high percentage of aromatics but is an oil having suitable boiling range and containing fractions which beneficially restore the asphalt to its original state. Typical gas oils which have been found highly effective for the present process are described in Examples 1—6 given hereinafter. A similar type of oil having a lower A. P. I. gravity and a higher boiling range is clarified oil. Both of these oils have aromatic contents which usually are above about 50% by weight. The thermally cracked stocks which are suitable as softeners for use in the present process are usually prepared by multiple cracking procedures wherein a previously cracked oil is subjected to further cracking steps until it has a sufficiently high aromatic content. The Edeleanu type of extracts usually have very high aromatic contents in the neighborhood of 70—80%. These may be used without modification or may be diluted down to the minimum effective aromatic concentration specified herein either with a non-aromatic oil or with one of the other preferred types of aromatic softeners.

The following examples are illustrative of preferred catalytically cracked gas oils which have proved to be effective softeners or conditioners for asphalt in paving compositions in accordance with my invention:

|                               | Example 1 | Example 2 | Example 3 | Example 4 | Example 5 | Example 6 |
|-------------------------------|-----------|-----------|-----------|-----------|-----------|-----------|
| Gravity, °A.P.I.              | 24.0      |           |           |           | 27.2      | 21.5      |
| Flash, °F.                    | 230       | 188       |           |           | 160       | 230       |
| Aromatic Content, Percent Wt. | 41        | 87        | 97.8      | 96.7      | 65        | 57.5      |
| Initial Boiling Point, °F.    | 508       | 390       | 440       | 546       | 385       | 460       |
| Final Boiling Point, °F.      | 736       | 630       | 620       | 706       | 500       | 694       |
| 10% Point, °F.                | 546       | 481       | 457       | 569       | 400       | 500       |
| 50% Point, °F.                | 596       | 525       | 478       | 588       | 423       | 644       |
| 90% Point, °F.                | 684       | 580       | 530       | 654       | 463       | 634       |
| Viscosity S.S.U. at 100° F.   | 47        | 35        |           |           |           | 39        |

a new surface. The principal difficulty with this method is that due to the basic difference in surface resistance of the relatively soft asphalt and the hard mineral aggregate with which it is combined, the two substances are very difficult to separate and break down to their original component sizes. This results in a rough, loosely bound surface which ravelles and disintegrates in a comparatively short time.

Another method which has been attempted is to add solvents, such as kerosene, diesel fuel, etc. to the surface material. This has been unsuccessful since the use of such solvents has resulted in stripping the asphalt from the aggregate and total destruction of the material as a surface-forming substance.

I have found that old and worn asphalt surfaces may be effectively reclaimed by using specific amounts of conditioners of the type described above, the amounts depending upon several factors, principally the amount and consistency of the worn asphaltic material, and the screen analysis of the aggregate present.

75 I have further found that the softener must be intimately mixed with the material to be reclaimed. In accordance with my invention this is accomplished by removing the worn asphaltic surface from the roadbed or other base and pulverizing or fracturing the material, mixing the material and simultaneously adding the conditioner in the desired proportions.

80 The following examples are illustrative of composi-

tions in accordance with my invention in the proportions by weight indicated:

*Example A*

|             | Parts |
|-------------|-------|
| Asphalt     | 185   |
| Conditioner | 51    |

In this example the asphalt recovered from the road surface was a soft asphalt having a penetration (at 77° F.) of 300 and the conditioner used corresponds to Example 6 above. It is to be understood in this and the following examples that the asphaltic material recovered from the road surface included a major proportion of a mineral aggregate such as sand and crushed rock. In Example A set forth above the screen analysis of the pulverized surface material was as follows:

| Screen size: | Percent passing |
|--------------|-----------------|
| 3/8"         | 100             |
| No. 4        | 99              |
| No. 8        | 98              |
| No. 16       | 96              |
| No. 30       | 86              |
| No. 50       | 71              |
| No. 100      | 55              |
| No. 200      | 44              |

It will be noted that the above analysis of the surface material indicates what is termed in the art "an extremely dense mixture." Due to the lack of adequate voids the stability of this composition as relaid was poor and therefore an amount (about 33%) of  $\frac{5}{16}$  to No. 8 crushed rock was added.

*Example B*

|             | Parts |
|-------------|-------|
| Asphalt     | 118   |
| Conditioner | 18    |

Here the asphalt recovered from the road surface had a penetration of 150 and the conditioner used corresponds to Example 6 above. The screen analysis of the pulverized surface material was:

| Screen size: | Percent passing |
|--------------|-----------------|
| 1"           | 100             |
| 3/8"         | 67              |
| No. 4        | 59              |
| No. 8        | 50              |
| No. 16       | 43              |
| No. 30       | 36              |
| No. 50       | 21              |
| No. 100      | 13              |
| No. 200      | 13              |

*Example C*

|             | Parts |
|-------------|-------|
| Asphalt     | 84    |
| Conditioner | 8.4   |

The asphalt component of this surface material had a penetration of 10 and the conditioner used corresponds to Example 6 above. The screen analysis of the pulverized surface material was:

| Screen size: | Percent passing |
|--------------|-----------------|
| 1"           | 100             |
| 3/8"         | 30              |
| No. 4        | 22              |
| No. 8        | 20              |
| No. 16       | 13              |
| No. 30       | 9               |
| No. 50       | 6               |
| No. 100      | 6               |
| No. 200      | 4               |

In carrying out my invention the first step is to analyze a representative sample of the surface material to be reclaimed. As will be apparent from the above example the amount of conditioner required depends principally upon the amount and grade of asphalt present, as well as the screen analysis of the surface material to be reclaimed. It is generally desirable in order to obtain maximum wearability to add only so much of the conditioner as is necessary to accomplish the desired softening action and to leave the proper amount of flux oils necessary to properly condition the mixture. It may be desirable to add new asphalt and/or more aggregate, depending upon the analysis of the used material as well as upon the properties desired in the new road surface it-

self, which latter properties are governed by contemplated traffic conditions, atmospheric conditions and the funds available. After the amount of conditioner required has been determined, and as indicated above this preferably will be in the range of 10-30% based on the asphalt present, the mixture may be designed in accordance with standard practices known to those skilled in the art in designing new road mixes.

The remainder of the process is carried out in the field. The old surface is first torn up by means of toothed scarifiers or rooters or the like. After the initial breaking up and uprooting has been accomplished the slabs of surface material, some of which are over two square yards in area, are reduced in size by heavy grid rollers. The rollers are followed by a conventional mobile combination feeder and rock breaker. These machines are provided with a conveyor belt which delivers the broken surface material from the road bed into a crusher or impact breaker of the revolving hammer type. One pass of this machine which deposits the crushed material in a windrow has been found to be generally sufficient to reduce the material substantially to the size of the original aggregate. Next, a conventional road mixer which is a self-propelled unit, including rotating drums mounted in tandem on which are placed staggered spades alternately angled to provide maximum mixing in addition to pulverizing, is passed over the windrow. The mixer is further provided with a series of spray nozzles through which the conditioner is introduced in a fine spray while the mixer is in operation. While not essential, it is very important that the conditioner is added simultaneously with the mixing so that the motion of the asphaltic particles will assure even distribution of the conditioner throughout the mix.

While the total amount of conditioner may be added in one pass of the road mixer I have found it preferable to add the conditioner in at least two portions to increase its effectiveness and to facilitate control by allowing visual inspection between additions. After the first application the material is thoroughly mixed, left in a windrow for at least several hours, and then the remaining amount of conditioner is applied in the same manner by use of the road mixer. At this point a rest period is provided to permit the conditioner to act upon the hard oxidized asphalt. This curing period will vary from a few hours to several days, depending upon weather conditions and the hardness of the asphalt upon which the conditioner must act. Experience has indicated that an average period of 48 hours is required.

After the material has been cured it is mixed thoroughly to blend and integrate the mixture. A sample of the finished mix is taken and analyzed as a check on the design and if found correct the surface may be completed by any of the accepted methods or the material may be stockpiled for future use.

I have found that the above described asphaltic conditioners may be advantageously employed in the construction of road surfaces, roofing, etc. with air-blown asphalt. The present practice is to ship solidified asphalt in barrels, and in order to render the material workable it is necessary to liquify it by heating before mixing with the aggregate. With the use of the conditioners described above the asphalt may be comminuted and furnished in sacks. This material may then be mixed cold with the conditioner and aggregate and laid without the use of the heat which is generally required.

While I have fully described preferred embodiments of my invention, it is to be understood that I do not wish to be limited to the details herein set forth, but my invention is of the following scope of the appended claims.

I claim:

1. A process for reclaiming used asphaltic surface material which includes the following steps: removing the material from its foundation; reducing the material in size; adding between about 10 and about 30 percent by weight, based on the asphalt content of the material, of a relatively non-volatile liquid hydrocarbon conditioner having an aromatic content of not less than approximately 40 percent by weight; thoroughly mixing the conditioner and asphaltic material; and curing the mix.

2. A process for reclaiming used asphaltic surface material which includes the following steps: removing the material from its foundation; reducing the material in size; adding a liquid hydrocarbon conditioner having an aromatic content of not less than approximately 40

percent by weight and boiling from about 400 to about 750° F.; thoroughly mixing the conditioner and asphaltic material; and curing the mix.

3. An asphaltic composition to be used for road surfaces and the like, comprising a major proportion of aggregate; a minor proportion of asphalt; and 10 to 30 percent by weight, based on the asphalt content of the material, of a liquid hydrocarbon conditioner having an aromatic content of not less than approximately 40 percent by weight and boiling from about 400 to about 750° F.

4. An asphaltic composition to be used for road surfaces and the like, comprising a major proportion of aggregate; a minor proportion of asphalt; and 10 to 30 percent by weight, based on the asphalt content of the material, of a relatively non-volatile liquid hydrocarbon conditioner having an aromatic content of not less than approximately 40 percent by weight.

5. An asphaltic composition to be used for road sur-

faces and the like, comprising a major proportion of aggregate; a minor proportion of blown asphalt; and 10 to 30 percent by weight, based on the asphalt content of the material, of a liquid hydrocarbon conditioner having an aromatic content of not less than approximately 40 percent by weight and boiling from about 400 to about 750° F.

**References Cited** in the file of this patent

**UNITED STATES PATENTS**

|           |          |                |
|-----------|----------|----------------|
| 657,799   | Varney   | Sept. 11, 1900 |
| 711,115   | Lober    | Oct. 14, 1902  |
| 760,051   | Amies    | May 17, 1904   |
| 2,308,245 | Ortynsky | Jan. 12, 1943  |

**FOREIGN PATENTS**

|         |               |               |
|---------|---------------|---------------|
| 16,657a | Great Britain | ----- of 1902 |
|---------|---------------|---------------|